

(No Model.)

2 Sheets—Sheet 1.

C. M. LUNGRREN.  
REFRACTORY FILAMENT FOR LIGHTING.

No. 365,832.

Patented July 5, 1887.



*Fig. 5.*



WITNESSES:

*Gabriel J. W. Gabler.*  
*Wm. T. Capel.*

*INVENTOR*  
*Chas. M. Lungren*

BY

*Townsend & Mar. Arthur*  
ATTORNEYS

(No Model.)

C. M. LUNGREN.

2 Sheets—Sheet 2.

REFRACTORY FILAMENT FOR LIGHTING.

No. 365,832.

Patented July 5, 1887.



WITNESSES:

*Gabriel J. W. Galster*  
*Wm. A. Cade*

INVENTOR

*Chas. M. Lungren*

BY

*Townsend & MacArthur*

ATTORNEYS

# UNITED STATES PATENT OFFICE.

CHARLES M. LUNGRÉN, OF NEW YORK, N. Y.

## REFRACTORY FILAMENT FOR LIGHTING.

SPECIFICATION forming part of Letters Patent No. 365,832, dated July 5, 1887.

Application filed August 12, 1885. Serial No. 174,233. (No model.)

*To all whom it may concern:*

Be it known that I, CHARLES M. LUNGRÉN, a citizen of the United States, and a resident of New York, in the county of New York and State 5 of New York, have invented a certain new and useful Refractory Filament for Lighting, of which the following is a specification.

This invention has reference to a filament or thread of the refractory earths—such as 10 lime, magnesia, zirconia, &c.—for use in producing light by means of its incandescence, by exposure to the heat of a non-luminous gas-flame; or the gas-flame may be that of a non-luminous gas—such as hydrogen, or a mixture 15 of hydrogen and carbonic oxide—or ordinary illuminating-gas with a proper admixture of air, or any of the volatile combustibles with which a non-luminous flame may be made. The flame may burn in the air under ordinary 20 pressure, or it may be supplied with air under pressure, and thus constitute a blow-pipe flame. In any case it is preferable to heat the air and the gas to increase the temperature of the flame, and consequently the brilliancy of the light.

In the drawings I have shown various forms in which the filaments may be used and some of the ways in which they may be combined with heating-burners for the purpose of producing light.

In Figure 1 I have shown two filaments, L and L', placed within the flame, F, of an ordinary bat-wing burner, b. The ends of the filaments are attached to platinum wires, 35 which are supported in the socket S.

In Fig. 2 the filamentary body is shown in the form of a fine spiral bent into ring shape. The burners shown in these two figures are designed to be used with fuel or non-luminous 40 gas.

In Fig. 3 is shown a form of burner in which a mixture of ordinary illuminating-gas and air is burned. It is provided with a wing-top, b, to give a flat flame, and the incandescent 45 refractory body is shown in the form of a fine spiral, as in Fig. 2.

In Fig. 4 there is shown the combination of a spiral with an atmospheric burner producing a cylindrical flame. B is the burner-tube, 50 from the mouth of which the mixed gas and air burn. F is the flame, and I an incandescent-spiral. The flame is shielded from

drafts by a chimney, G, which rests in the holder G', formed by the upper end of the air-casing surrounding the lower portion of 55 B. The spiral is shown as supported at its lower end in the holder S. It may, however, be hung from the top of the chimney G or be attached to it by suitable supports, as described in the United States Patent to me, 60 No. 336,576, granted February 23, 1886.

In Fig. 5 the incandescent body is shown in the form of a cylindrical net-work, and in Figs. 6 and 7 in the form of a flattened net-work to adapt it to a flat form of flame.

It is not necessary that the filaments be bent into a curved form, as they may be straight and a number of them grouped together to form a sufficient incandescent surface. Several forms of such construction are shown in 70 Fig. 8.

In Fig. 8 is shown a number of filaments arranged to form a cylindrical structure, within which the flame of the Bunsen burner B burns. They are curved in at their upper ends to a 75 common point, as shown.

Various other forms of burners and disposition of the filaments may be used; but the above are sufficient to show the variety of ways in which the filaments may be employed 80 for the purpose of carrying out my invention.

It is not my purpose to claim in this application any arrangement of filamentary bodies with heating appliances for the purpose of 85 producing light, as these will form the subject-matter of other applications.

I confine myself in my present application to such filament *per se* and the method of manufacturing the same, in pursuance of the 90 reservation contained in a prior application filed June 6, 1881, in which such invention was described but not claimed. In making such filament I prepare a plastic mass of any of the above materials or mixtures of them by 95 kneading them with water, or, preferably, a solution of a mucilaginous binding material, such as glue or gum, or other combustible material, which will be consumed in the further treatment of the filament. When the mass is 100 of the proper consistence, it is put in a press and the filament obtained by expressing the material through a die.

Immediately after their formation, while

they are still moist, the filaments should be bent into the required shape. The method for doing this will vary with the shape. A simple bow or loop may be formed by bending 5 or coiling the material in a mold of absorbent material, such as plaster-of-paris dusted over with plumbago. After removal from the mold the filaments may be thoroughly dried by being placed between layers of absorbent material, such as blotting-paper.

In making a spiral the filaments are coiled around a mandrel, which is preferably of wood rubbed with plumbago to prevent adherence of the coil, and allowed to dry upon it. This 15 they will do without warping or cracking, if the plastic material is of the proper consistency.

In forming a curved spiral, such as that shown in Fig. 2, the filament may be coiled 20 upon a curved mandrel or coiled upon a straight flexible mandrel, which is then bent to the desired shape while the filament is still moist.

In making a net-work, such as that shown in 25 Fig. 6, the filament is coiled on a mandrel in the form of a double spiral, the threads adhering to each other where they cross.

At the completion of the drying process the 30 filaments are ready to be burned, by which means they become hard and dense and suitable for the purpose of incandescence.

A plain bow or loop may be burned directly in a flame by applying the heat gradually and finally carrying it to the highest attainable temperature. A spiral or other 35 cylindrical form is best burned in a mold heated to a high temperature in a blast-furnace. The spiral is placed upon a rod of highly-refractory material—such as lime or magnesia—supported horizontally in a tubular mold. The central pencil and its encircling coil are raised to a high temperature by radiation from the wall of the inclosing mold. The carbon of the 40 material is in this operation burned out and the filament hardened.

The supporting-pencil should be of such a size as to allow of a shrinkage of the spiral, and it is best to subject the spiral to several burnings supported on successively smaller 45 pencils. After removal from the mold, if not sufficiently hard, the spiral may be further

burned in the flame, but still being supported on a center. A bow or loop may also be burned in a mold by being formed as a part of a close-coil spiral. This spiral is then burned as above described and afterward cut up into sections to form bows.

Filaments prepared in this manner are hard and dense, have a polished surface, and when fine are slightly translucent, the vitrification 60 extending throughout them. They may be produced of almost any desired fineness, and when sufficiently heated emit a clear white light.

I do not specifically claim in this application 65 the various ways of combining the filamentary body of refractory earth, herein shown and described, with heating appliances for the purpose of raising said body to incandescence, as my inventions in that respect are made the subject of other applications, and particularly of 70 a pending application filed by me December 26, 1885, Serial No. 186,699.

I do not herein claim the method of forming filamentary bodies of refractory earth, 75 which consists in first forming a filamentary body composed of a combustible binding material and a refractory material, and then burning out the binding material, as that part of my invention forms the subject of a divisional 80 application filed June 8, 1887, Serial No. 240,572.

What I claim as my invention is—

1. An incandescing organ for gas or other burners, consisting of a filamentary body of 85 refractory earth, such as lime, magnesia, zirconia, and the like.

2. An incandescing organ for gas or other burners, consisting of a filamentary body of refractory earth—such as lime, magnesia, zirconia, and the like—made by expressing the material from a plastic mass in the form of fine threads and then forming these into a filamentary structure of the desired shape or form.

Signed at Philadelphia, in the county of Philadelphia and State of Pennsylvania, this 95 7th day of August, A. D. 1885.

CHARLES M. LUNGREN.

Witnesses:

ALBERT W. COX,  
CHARLES CARVER.